

Nov. 17, 1936.

R. W. SPRINGER

2,060,952

POLISHING WHEEL

Filed May 23, 1935



Fig. 1



Fig. 2



Fig. 3

INVENTOR.  
Ray W. Springer

BY  
Parker & Burton  
ATTORNEYS

## UNITED STATES PATENT OFFICE

2,060,952

## POLISHING WHEEL

Ray W. Springer, Detroit, Mich.

Application May 23, 1935, Serial No. 22,937

9 Claims. (Cl. 51—193)

My invention relates to improvements in polishing wheels and particularly to an improved wheel body to the circumference of which is secured the abrasive compound that forms the 5 polishing surface.

My improvement relates particularly to that type of polishing wheel which is built up of several laminations of fibrous sheet material such as woven fabric or the like suitably secured together. Preferably I employ a fabric of a loosely woven coarse character, such as woven jute. I propose to secure these several laminations of the fabric together without stitching or other securing means to form a compact integral wheel body which possesses long wearing properties and which is sufficiently resilient to absorb the shock and pressure application of work applied to its periphery without resulting in permanent deformation.

My improved polishing wheel is structurally uniform throughout. When the polishing face with which wheels of this type are provided has worn down, necessitating the application of a new face thereto, and the wheel is trued up to receive such new face, the wheel, at such new diameter, will possess the same normal resiliency as it possessed at its original diameter. Furthermore, it is free from the hard places which are found along the lines of stitching in wheels where the fabric laminations are stitched together.

An important characteristic of my improved wheel is that the body structure formed of the plurality of laminations of woven fabric or the like constitutes a structurally unitary body. These several laminations are secured together by a latex compound which is supplied in such a quantity as to comprise substantially one-half by weight of the entire wheel body. The latex compound is of such a character that it possesses a normally permanent resiliency co-extensive with the normal life of the wheel body. The latex compound carries an antioxidant which renders it normally permanently tacky and prevents aging of the rubber content. It extends throughout the entire structure securing the several fabric laminations together and extends as a film over the threads of the individual laminations filling the interstices therebetween and forming a continuous resilient connective structure through the interstices of the laminations and between the laminations. It forms a moisture resistant film enclosing the individual fibers which make up the several fabric layers.

An object is to provide such a wheel body which will be inexpensive, easily fabricated, of an inte-

gral unitary character, sufficiently rigid and sturdy to fulfill the intended function thereof, and which has a circumferential portion of sufficient resiliency and pliability to yield without resulting permanent deformation under the 5 stresses received during use. This yielding circumferential portion forms a unitary construction with and is an integral part of a central portion, which central portion is sufficiently rigid to support and carry the yielding circumferential portion.

An important feature is that my improved polishing wheel possessing the above recited characteristics is formed of a plurality of laminations of flexible sheet material, such as woven fabric, 15 adhesively secured together by a yielding resilient binder; and the central portion of the wheel body immediately surrounding the axis of the wheel body is compressed to the point of substantial rigidity, while the outer portion adjacent to the circumference is compressed to a substantially less degree, whereby it possesses resiliency and is normally compressible and yielding.

Other objects, advantages, and meritorious features will more fully appear from the following description, appended claims and accompanying drawing, wherein:

Figure 1 is a side elevation of a polishing wheel embodying my invention,

Fig. 2 is an elevation taken at right angles to the view of Fig. 1, and partly broken away to show the structure in section, and

Fig. 3 is an elevation partly in section of one of the composite laminations which go to make up my improved wheel.

Polishing wheels of this general character have heretofore been fabricated of a plurality of fabric disks sewed together and then provided upon the periphery of the wheel body with a layer or band of abrasive suitably deposited or secured thereon. This application forms a continuation in part of my application Serial No. 699,859.

In the structure of the instant application I employ fabric sheet material cut into disks. A plurality of these disks are adhesively secured together to form a composite lamination 10. One of these laminations is shown in Fig. 3. The separate sheet disks may be adhesively secured together by a suitable composition latex binder. Loosely woven cloth such as burlap may be used to form the disks. The binder extends through the interstices of the several disks, thoroughly impregnating them forming a moisture resistant film enclosing the individual fibers which make up the several layers and adhesively securing the 55

several layers together. The binder also forms a film between the separate disks. The latex compound used is such that it is adapted to normally permanently retain its yielding resiliency. By 5 latex compound I mean a water emulsion of rubber which comprises the natural product latex, modifications or compounds thereof, or artificial aqueous dispersions of rubber. In Fig. 3 I have shown five separate disks so secured together. 10 Any suitable number may be used. In practice such number as was required to make up the wheel body would be employed.

In order to form the wheel body I superimpose a plurality of these separate impregnated laminations. 15 This pile of laminations is placed in a suitable press and subjected to the required pressure to press them tightly together. The pressure used may be such as to reduce the thickness of the laminations one half. The press is so formed that a central or axial portion 12 of the wheel body is compressed to a greater degree than the circumferential portion 14 and the pressure is such that this axial portion is rendered substantially rigid and constitutes a substantially inflexible supporting portion which carries the integral circumferential portion 14, which, not having been subjected to as great pressure, possesses sufficient resiliency to yield to the shocks which the wheel body receives during use without 20 breakage or permanent deformation. The abrasive is secured to the periphery of the portion 14 in a suitable manner.

When the abrasive wears down the wheel may be trued up and a new coating of abrasive secured upon the periphery. The circumferential abrasive supporting portion of greater diameter possesses a uniform yielding character from the first. This attribute persists throughout the life 30 of the wheel body. Due to the fabrication of a wheel body in this form and after the herein described fashion, the circumferential abrasive supporting portion yields to the desired degree as herein described, yet it is supported by the relatively rigid axial portion so that the wheel runs true and does not yieldingly deform under normal pressure except within the desired radial 40 limits as described, and does not deform axially by bending or the like but is held by the relatively inflexible central portion against such deformation.

The several sheets are thoroughly impregnated with the latex compound and the compound passes into the interstices of the sheets. The material is of such a character and the carrying 50 out of the process is such that the weight of the completed body will be made up approximately equally of the sheet material and compound. During the compression of the sheets together the latex compound is driven through the interstices of the several sheets to such an extent that it forms a continuous normally resilient relatively tacky connective tissue or structure extending radially and axially throughout the entire body. It extends as a connecting structure through the 60 interstices of the several sheets connecting them together. The pressure is exerted also to such a point that the resulting body has an axial dimension approximately one half of that of the uncompressed pile of sheets. The wheel is preferably not vulcanized and the binder retains its tacky character. In Fig. 2 I show such a body structure as it would appear complete but with sheets exaggerated in thickness. In this figure 70 there is also shown a polishing face 16 about the

periphery of the wheel body. The particular polishing face forms no part of my invention.

I employ a compound which will retain its resiliency for the normal life of the body structure and which might therefore be termed "permanently resilient". The compound also must not deteriorate with age and it must withstand the heat and other temperature changes throughout such a range as will be met with in the operation of the wheel. I propose to use a suitable rubber 10 latex compound which possesses these desired characteristics. A compound which has been found satisfactory comprises: 50 c. c. m. of rubber latex, 4 c. c. m. of saturated Burgandy pitch solution, and 20 drops of Neozone L. 15

The Burgandy pitch may be varied up to 6 c. c. m. with the amount of latex above set forth and the Neozone L may be increased up to sixty drops in the formula. The pitch solution may be formed by dissolving the pitch in ammonia or some other suitable solvent to the maximum capacity of the solvent. The Neozone L is a commercial product and is an anti-oxidant. Other similar suitable anti-oxidants might be employed. It prevents injurious aging of the compound and preserves its tacky condition so that the laminations will remain united or will reunite following an opening up of the layers. The pitch tends to impart and to permanently preserve the tacky characteristic of the compound. 30

It will be found that the wheel body, when compressed, possesses an inherent resiliency which will permit it to withstand considerable shock of work being urged thereagainst without permanent deformation or development of an out-of-round condition. This resiliency is uniform as its structural character is uniform and continues throughout the normal life of the wheel. The tensile strength of the fibers is 40 increased approximately one-half by the compound and the compound likewise eliminates the tendency of the fibers to break, crack, or flake off under the action of pressure thereagainst.

What I claim is:

1. A polishing wheel body formed of a plurality of loosely, coarsely woven fibrous disks impregnated with a normally permanently tacky and resilient adhesive moisture resistant binder, said disks being compressed together into an integral wheel body with the binder filling the interstices of the disks and adhesively securing them together. 50

2. A polishing wheel body formed of a plurality of loosely, coarsely woven fibrous disks impregnated with a normally permanently tacky and resilient adhesive moisture resistant binder, said disks being compressed together into an integral wheel body with the binder filling the interstices of the disks and forming a covering surrounding the individual fibers thereof, and adhesively securing the disks together, said binder being resistant to oxidation and constituting substantially one half by weight of the wheel body. 60

3. A polishing wheel body comprising a plurality of fabric layers impregnated with an anti-oxidant latex composition binder filling the interstices thereof and rendering the individual fibers moisture resistant, said layers being compacted and adhesively secured together into an integral body, said binder forming a connective structure extending throughout the body and being substantially permanently resilient and tacky, said plurality of disks being compressed so 70

as to have an axial portion of substantially less diameter than the wheel body compressed to a substantially less axial dimension and greater rigidity than the peripheral portion of the wheel.

5. A polishing wheel body comprising a plurality of fabric layers impregnated with an anti-oxidant latex composition binder filling the interstices thereof and rendering the individual fibers moisture resistant, said layers being adhesively secured together and compacted throughout the peripheral portion of the wheel body to substantially one half the uncompressed thickness of the plurality of layers while retaining substantial yielding resiliency, said wheel having 10 its axial portion compacted to a substantially greater degree than the peripheral portion and into substantial rigidity.

5. A polishing wheel body consisting of a plurality of loosely integrated fibrous discs impregnated with and adhesively secured together in compacted juxtaposition by a normally permanently tacky and resilient latex compound.

6. A polishing wheel body consisting of a plurality of loosely integrated fibrous discs impregnated with a latex compound carrying a pitch 25 ingredient rendering the compound normally

tacky, said discs being adhesively secured and compacted together.

7. A polishing wheel body formed of a plurality of fibrous discs adhesively secured compacted together and having the individual fibers which 5 make up the several discs adhesively secured together by a normally tacky and resilient latex compound.

8. A polishing wheel body consisting of a plurality of loosely integrated fibrous discs impregnated with and adhesively secured compacted together by a normally tacky resilient latex compound, said compound being uniformly distributed throughout the wheel body holding the 10 fibers which make up the same resiliently together and preventing separation or fraying 15 thereof.

9. A polishing wheel body consisting of a plurality of loosely integrated fibrous discs impregnated with and adhesively secured together in 20 compacted juxtaposition by a normally permanently tacky and resilient latex compound, said wheel body having a portion adjacent to its axis of substantially greater density and less yielding than the portion adjacent to its periphery. 25

RAY W. SPRINGER.